

H. B. WEAVER & J. GAYLEY,  
BLAST FURNACE PRACTICE.  
APPLICATION FILED AUG. 8, 1918.

1,292,937.

Patented Jan. 28, 1919.

2 SHEETS—SHEET 1.



Inventors,  
Harry B. Weaver,  
James Gayley,  
By their Attorneys  
Fannie, Davis, Marvin & Goulds

H. B. WEAVER & J. GAYLEY,  
BLAST FURNACE PRACTICE,  
APPLICATION FILED AUG. 8, 1918.

1,292,937.

Patented Jan. 28, 1919.

2 SHEETS—SHEET 2.

Fig. 2.



Fig. 3.



Inventors:  
Harry B. Weaver,  
James Gayley,  
By Their Attorneys  
Fannie Davis, Marvin Edwards.

# UNITED STATES PATENT OFFICE.

HARRY B. WEAVER, OF CATASAUQUA, PENNSYLVANIA, AND JAMES GAYLEY, OF NEW YORK, N. Y.

## BLAST-FURNACE PRACTICE.

1,292,937.

Specification of Letters Patent.

Patented Jan. 28, 1919.

Application filed August 8, 1918. Serial No. 248,838.

To all whom it may concern:

Be it known that we, HARRY B. WEAVER, a citizen of the United States, residing at Catasauqua, Lehigh county, State of Pennsylvania, and JAMES GAYLEY, a citizen of the United States, residing at No. 555 Park avenue, in the city, county, and State of New York, have invented certain new and useful Improvements in Blast-Furnace Practice; 10 and we do hereby declare the following to be a full, clear and exact description of the invention, such as will enable others skilled in the art to which it appertains to make and use the same.

15 The constituents of the customary charges regularly fed into an iron blast furnace consist of iron ore, limestone and coke, and contain varying percentages of alkali compounds, *i. e.*, compounds of potassium and sodium. Descending in the furnace from a colder to a hotter temperature these alkali compounds encounter the highest temperature in the zone of combustion in the neighborhood of the twy whole where the heated air 20 blast comes in contact with the incandescent fuel, and an important chemical reaction results.

The carbon of the coke and the nitrogen of the air blast cannot combine at the existing temperature without the aid of an intermediary. The alkali-metals found in the furnace provide the most effective medium for bringing the nitrogen and carbon into combination in the combustion zone and 35 are present in said zone. The fact that potassium cyanid is formed in the blast furnace has been known, in fact, for a long time, but has been regarded merely as an interesting chemical phenomenon, and, in so far 40 as we are aware, it has not been known that it exists in the blast furnace in sufficient quantity to make it available for any useful purpose, nor that there were any other like compounds present whose withdrawal would 45 be feasible without detriment to the blast furnace operation, where certain essential conditions must be maintained in order to permit the furnace to discharge its required functions in the production of its prescribed 50 metallurgical product, that is to say, (in a pig-iron blast furnace) its output of pig iron.

The present invention is based upon the

discovery that, in addition to potassium cyanid, there are present in the furnace gases, 55 at and in the neighborhood of the twy whole, other compounds in which the alkali metals are associated, and that the potassium cyanid and these other compounds are present in such quantity in the furnace and in such association with the reducing gases constantly rising from the zone of intense combustion at or near the twy whole that it is feasible and remunerative to withdraw from the furnace a portion of the said reducing gases and to 60 abstract therefrom by condensation or otherwise the compounds of the alkali metals so as to recover them in large quantity for useful purposes, and without diverting from the blast furnace any such amount of the 65 reducing gases as are required for serving their preparatory function for the charge in the upper part of the furnace shaft. Accordingly, the invention provides an operation wherein the blast furnace delivers its 70 normal output of pig iron and a normal slag, preserves the necessary conditions for the required reactions in the combustion zone, permits the reducing gases rising from the combustion zone to exercise the required reducing 75 action in the furnace shaft, and, coincident with these several necessary provisions for the successful operation of the iron blast furnace, permits the withdrawal and recovery, on a commercial scale, of highly valuable 80 compounds of the alkali metals, some of which were not known to exist in the combustion zone of the blast furnace and which, in their entirety, were not known to be present in sufficient quantity to justify an attempt to remove them, or that paying quantities of any of such compounds were recoverable while still preserving standard blast 85 furnace conditions.

The recovery of these valuable constituents, in an effective way, and without detriment to the normal functioning of the blast furnace is dependent upon factors of the furnace operation which we have taken into careful account in working out the practice 90 constituting the subject-matter of the present invention.

Thus, the compounds of the alkali metals with carbon and nitrogen are formed, as hereinbefore indicated, in the zone of combustion in the neighborhood of the twy whole,

where the heated air blast comes in contact with the incandescent fuel. On their formation, they pass upward in the furnace with the large volume of reducing gases, thus meeting the colder charges of materials which are descending. Upon entering these colder charges, the alkali metals are precipitated and are returned again to the combustion zone. So, also, the potassium cyanid, passing upward in the furnace, reaches a point where the combination is broken so that only an insignificant portion thereof passes out with the exit gases.

It is essential, therefore, that the potassium cyanid and other compounds of the alkali metals whose recovery is desired, be withdrawn from the zone where they are produced and before any important precipitation or disintegration takes place in their upward travel. This zone of production is located in the neighborhood of and in close proximity to the twyers, and, if the vaporized compounds are not withdrawn at or near their place of formation, they are lost. The purpose of the present invention is to prevent such loss, and to recover the products for useful purposes.

Accordingly, in carrying out the invention, a portion of the reducing gases containing a corresponding quantity of the vaporized compounds is withdrawn from the furnace at a point in the neighborhood of the twyers, and preferably above them, care being taken to restrict the quantity of the gases withdrawn to an amount which will not interfere with the requirements of the reducing gases in the upper zone or shaft of the blast furnace. The furnace operator is enabled to judge of the limitations in this regard, by noting, from time to time, the character and particularly the color of the slag, which he may tap off, for that purpose, as a governing test, at intervals, at the cinder notch of the blast furnace.

This slag (in a pig-iron blast furnace) should normally be gray or white in color, thus indicating that only minute quantities of iron appear in the slag, and that the blast furnace is acting under proper conditions which require that practically all of the iron in the carefully calculated ingredients of the charge shall be recovered in the metal output of the furnace as pig iron.

If the operator finds that the slag substantially retains its normal gray or white color and substantially its normal temperature and fluidity, he will know that the amount of the reducing gases withdrawn is within the limits that can be tolerated for acceptable blast furnace conditions, and also that the formation of the recoverable alkali metal compounds is progressing normally in the combustion zone. If, on the other hand, he finds that the slag, in the test tap, has assumed or is beginning to assume an

abnormal darker tint, indicative of the passage of oxid of iron into the slag, he will be advised that the necessary conditions for the proper functioning of the blast furnace are being interfered with by an excessive withdrawal of the reducing gases, and also that the formation, composition, and output of the desired condensable products are suffering abnormal irregularities, correspondingly interfering with the intent and purposes of the invention. He will, accordingly, be able to correct the irregularities referred to, by appropriately limiting or restricting the amount of the reducing gas withdrawn, per unit of time, or by temporarily restoring, either wholly or partially, the usual blast furnace conditions, until the taking of a test at the cinder notch shows that the slag has been brought back to normal.

In some instances, the operator may prefer to withdraw continuously the portion of the reducing gases which it is found feasible to abstract for the recovery of the compounds of alkali metals recoverable without interfering with the necessary conditions of the blast furnace operation. In other cases, the operator may effect the withdrawal of such quantities of the reducing gases, at intervals. Either of these modes of operation are within the broad purview of the intended practice. Continuous or practically continuous withdrawal of the gases will be more advisable, in those instances where the quantity of alkali in the charge is relatively large. Intermittent withdrawal is to be recommended where the quantity of alkali in the charge is relatively small,—the large capacity of the blast furnaces, with the high heats employed and the perfect reduction of the ores, causing even the ordinarily small content of alkali in the charge to accumulate in considerable quantity, and it may thus build up gradually in succeeding time periods, so as to make it feasible and even desirable to remove it periodically at suitable intervals apart. Moreover, by the intermittent instead of the continuous withdrawal of the gas, furnace gas for the stack will be correspondingly conserved, thereby affording a wider safety factor for the blast furnace operation as a whole. It will also be understood that the recovery of the potassium cyanid and other alkali metal compounds contained in the withdrawn gases may be effected in any of the methods known to the art; that is to say, either by condensation, settling, screening, solution, electric precipitation, or the like, as will readily occur to those skilled in the art.

The withdrawal of the gases containing the products to be recovered in accordance with our invention may be through apertured plates or blocks inserted in the fur-

70

75

80

85

90

95

100

105

110

115

120

125

130

nace wall and provided with a water-cooled passageway. To each of these plates or blocks is connected a conduit pipe leading to the condensing or recovering apparatus.

- 5 In order to avoid condensation of the condensable material in the conduit pipe it may have a heat-insulating jacket either on the inside or on the outside, but if the insulation is on the inside it should be of a material 70  
10 resistant to the action of the gases and the vaporized compounds carried thereby.

The condensing may be conducted in one or more chambers and in one or more units 15 as may be desired. Where the withdrawal of the gases is to take place continuously, it is necessary to have more than one set of chambers or units, so that when one set is being cleaned, another set is available for 20 operation. After the gases pass through the condensing apparatus, they are preferably led through a flue of suitable length to permit them to cool down to a relatively low temperature whereupon they are led 25 through a filter, such as a bag filter, or other analogous apparatus, for the further removal of the fume which carries values. In passing through the condensing apparatus, the gases will be reduced in temperature, but if not sufficiently reduced in temperature to be led immediately to the filter, their passage through the flue above referred to, or through any like device, may be resorted to, as will be readily understood.

- 30 35 The final exit gas from the recovery apparatus, practically freed of its solid material, is not returned to the shaft of the furnace, inasmuch as the introduction of relatively cold gas into the hot gases within the 40 furnace would accomplish no useful purpose, and would even be deleterious for the reason that it would absorb heat. Accordingly, the final exit gas may either be wasted or may be led by a conduit to the stoves or 45 boilers of the plant for heating purposes, as the necessities of the plant may require, or it can be put to other appropriate uses.

The air supplied to a blast furnace usually enters the tuyers at a pressure of from 50 10 to 20 pounds per square inch. Accordingly, the pressure existing within the furnace will, in most instances, suffice for insuring the outflow of the portion of the gases to be withdrawn therefrom, and this 55 outflow may conveniently be controlled by an adjustable valve or damper at the outlet of the condensing apparatus, the rate of outflow of the withdrawn gases being so adjusted that the composition of the usual exit 60 gases from the furnace top is not appreciably changed.

Referring further to the uses and practice of the invention, we may take, as an example thereof, an average type of pig-iron blast 65 furnace producing 400 tons of pig iron

daily. In such a blast furnace there will be consumed daily approximately 1300 tons of coke, ore and limestone, so that a relatively small content of alkali in this aggregate will amount, in a day's operation, to a considerable quantity, and may be withdrawn by the practice of the present invention, at a rate appropriate to the alkali contents of the material charged.

In a given instance, the charge of a blast 75 furnace showed on analysis an average of potash (calculated as  $K_2O$ ) 0.28%, and an average of soda (calculated as  $Na_2O$ ) 0.55%. These contents of potash and soda amounted per ton of iron produced to 22 pounds of 80 potash and 35 pounds of soda. Such a furnace charge can be enriched in potash, if desired, by the addition of a potash-containing mineral, such as green sand (usually containing about 8% of potash), provided 85 the furnace operations are not disturbed from their proper function of producing pig iron, including the proper reduction of the iron ore, as indicated by the gray or white color of the slag. As hereinbefore 90 noted, a small amount of iron oxid in the slag suffices to turn it black, thereby indicating abnormally low temperature conditions in the furnace. Moreover, such a slag is necessarily an oxidizing slag, and its presence in the furnace tends to prevent the formation of cyanogen compounds which are among the most powerful reducing agents known,—so that the production of a black 95 or oxidizing slag of itself indicates conditions in the furnace that are unfavorable to the production of some of the compounds which it is the purpose of the invention to recover.

The accompanying drawings illustrate certain forms of apparatus adapted for carrying out the described invention.

In the drawings.—

Figure 1 represents, in vertical section, an iron blast furnace, and shows, in elevation, a suitable condensing system for the recovery of the alkali-metal and nitrogen compounds;

Fig. 2 represents a similar view showing a modified communication of piping between the blast furnace and the first chamber of the condensing system;

Fig. 3 represents a sectional plan view of Fig. 2.

Referring to the drawings, 3 represents a 120 pig-iron blast furnace, which, as ordinarily constructed, is from 80 to 100 ft. high. 4 represents the tuyers for the admission of the hot air blast, 5 the slag outlet or notch, and 6 the iron notch. 7 represents cooled 125 plates or blocks inserted in the hearth and bosh wall of the furnace, through which the portion of the reducing gases which it is permissible to remove without disturbing the essential blast furnace conditions are 130

withdrawn together with their content of the compounds of the alkali metals which are to be recovered.

The points of withdrawal of the gases are not limited to the particular location of any of the plates or blocks shown, but may be at any point in the wall inclosing the combustion zone. Thus, as indicated in Fig. 3, they may be spaced at substantially equal distances apart around the periphery of the furnace, and may all lead to the same initial chamber of the condenser system; in such case, instead of connecting the several blocks to a common bustle-pipe, individual pipes 9<sup>a</sup> will connect them severally, in straight-line direction, to the condenser chamber, so that it will be correspondingly convenient to remove any possible obstructions that might condense or otherwise form therein, and so that any individual pipe may be readily removed when occasion may require and substituted by another.

In all instances, the pipes making connection with the plates or blocks should be appropriately heat-insulated, either exteriorly or interiorly, or both, so as to appropriately resist the intense heat of the withdrawn gases, and, as hereinbefore stated, the lining chosen for the interior of the pipes should be of a character to resist the corrosive action of the alkali-metal compounds.

In the form shown in Fig. 1, the several plates or blocks make connection to a conduit 9, leading to the first condensing chamber 10 of the condensing system. The several blocks may, as shown in said figure, be connected to a manifold 8, for convenience and compactness of apparatus, instead of being connected directly to the conduit 9 without using the manifold.

The gases entering the condenser 10, at an opening 11, deposit the heavier and more readily condensable products therein and pass out through an outlet 12. In the construction of chamber 10, a water-container 13, which may be kept supplied from any convenient source of water (as, for instance, the valved pipe 13<sup>a</sup>) is so arranged that the water supplied thereto will flow over the upper edge of the container and down over the periphery of chamber 10, thereby cooling the gases within the chamber correspondingly and accelerating the condensation thereof. The waste water is collected in a gutter 14 at the lower part of the chamber 10 and flows off to waste at the discharge lip 15. 16 is an air valve which permits the air in the chamber 10 to escape when the gases are admitted to the chamber. 17 are lugs for lifting the chamber from its position, when desired, and substituting a fresh chamber, and, for this purpose, the joints 18 and 19 in the piping should preferably be ball joints. Valves 20 and 21 are used for regulating the flow of the gas.

The gas passes from chamber 10 through conduit 22 into chamber 23, which may also be water-cooled and wherein a further condensation of the condensable compounds takes place, and at a lower temperature than in chamber 10. The material condensed in chamber 23 may be removed at the hopper bottom which has an aperture provided with a suitable valve, as, for instance, the conical pivoted and counter-weighted valve 24.

The velocity of the gases in the chamber 23 is comparatively low so that a considerable quantity of the condensable compounds is recovered in said chamber. From the chamber 23, the gases next pass through the conduit 25, their flow being controlled by the adjustable valve 26. The conduit 25 conducts the gases to a bag filter or similar effective device in chamber 27. The bag filter 28 will remove practically all of the remaining compounds which are carried along in suspension by the gases. The bag filter is provided with a ring 32 connected thereto, and operating handles 29 extend through the walls of the chamber so that the workmen may shake the bag filter by means of these handles, thereby dislodging the material within the bag which material thereupon falls into the receptacle 30. The gases, after having passed through the filter, make their exit at 31 and can be carried off to any convenient place of use.

It will be noted that the exit pipes from the chambers 10 and 23 extend down to the lower portion of said chambers, so as to give the gases a longer path to travel before taking their exit therefrom. In passing from the chamber 23 to the chamber 27, the gas must be so far lowered in temperature that it will not consume or injuriously affect the material of the filter bag. This can be done by cooling the conduit 25 in any appropriate manner, as, for instance, by water jets externally applied thereto, or, (in substitution or connection therewith) by extending the length of the conduit so that the gases will have a sufficient length of travel to effect the necessary reduction in temperature.

The condensing system illustrated is typical of many others that might be substituted therefor. The quickly condensable compounds, which are heavier, are deposited in chamber 10. Those that are lighter and require further cooling, are deposited in chamber 23, and the compounds in suspension are recovered in chamber 27. The condensation and collection of the compounds may therefore be said to be fractional, and the temperature of the gases is lowered successively from one chamber to another to permit this fractional recovery of the compounds.

A typical instance will illustrate the practical results obtained by the practice of the invention. Thus, operations were conducted

on a pig-iron blast furnace 80 ft. high and 17 ft. 6 in. in diameter at the bosh and with a hearth 11 ft. 6 in. The data for a week's operation of this furnace were as follows:

- 5 Pig iron produced----- 1,450 tons.  
 Coke consumption per ton of  
 pig iron ----- 2,748 lbs.  
 Raw material used:  
 10      Ore ----- 2,623 tons  
       Coke ----- 1,982 tons.  
       Stone----- 993 tons.  
 Yield of ore mixture ----- 55.30 per cent.  
 Volume of air blast per minute=23,000 cu. ft.  
 15 Temperature of air blast 1200-1300 degrees  
       Fahr.

30 per cent. of the ore charge was Lake Superior ores, and 70 per cent. New Jersey magnetites. The vaporized compounds of 20 the alkali metals were withdrawn from a point above the twyers and led to a condensing apparatus, and from there to a bag filter.

The material collected in that part of the 25 apparatus preceding the filter was found, on analysis, to give the following percentages of potassium cyanid and other alkali metal compounds, to wit:

- 30      Potassium cyanid (KCN)=24.35%.  
       Carbonate of potash (K<sub>2</sub>CO<sub>3</sub>)=31.27%.  
 Soda (Na<sub>2</sub>O)=4.50%.

The material obtained from the filter portion of the apparatus gave the following percentages of potassium cyanid and other alkali-metal compounds, to wit:

- 35      Potassium cyanid (KCN)=49.05%.  
       Carbonate of potash (K<sub>2</sub>CO<sub>3</sub>)=24.95%.  
       Soda (Na<sub>2</sub>O)=6.20%.

These analyses illustrate the commercial and industrial capabilities of the invention.

40 They also illustrate, in a striking manner, the fact hereinbefore indicated, that there are present in the hearth and bosh of the iron blast furnace not only alkali cyanid but other compounds in which the alkali metals are associated, and that these are 45 there present in large quantity and in recoverable form as potassium carbonate, and also as sodium compounds (calculated as (Na<sub>2</sub>O)). In so far as we are aware, even 50 the presence of these additional compounds, as such, in the combustion zone of the iron blast furnace, has never before been established, nor their recovery effected.

It will, of course, be understood that by 55 the expression "iron blast furnaces" as used in the claims, we do not intend to exclude iron blast furnaces whose product may vary from pig iron, inasmuch as the blast furnace charge is frequently made up in such manner as to result in a product containing notable quantities of alloying metals, such as manganese, silicon, or the like.

In further explanation of the characteristic feature of the present invention, we may 60 point out that, in blast furnace practice, it is

absolutely necessary to maintain the thermal equilibrium or heat balance, which is relatively sensitive, in order to obtain the standard metal product of the blast furnace operation. The thermal equilibrium can, perhaps, best be understood from the point of view that the blast furnace consists of two separate pieces of apparatus, the one superimposed upon the other; the upper apparatus, is that in which occur the preheating 70 and reduction of the iron ore and other ingredients of the charge, while the lower apparatus is the hearth and bosh, in which the melting of the iron and cinder and the removal of the final traces of oxygen, etc., are 75 carried on, these being operations which can only occur at a certain (high) critical temperature.

The gas resulting from the combustion of the fuel in the lower apparatus must supply the heat necessary for both sets of reactions, or the furnace will not function according to its prescribed intent.

It so happens that the ordinary heat requirements of these two pieces of apparatus 90 are proportioned to one another in approximately the same relations as the heat available from the gases of combustion. These gases yield a small quantity of high temperature heat in cooling from their theoretical combustion temperature to the critical temperature, and a much larger quantity of heat in cooling from the critical temperature to the temperature at which they are discharged. There is generally an excess 100 for the latter purpose; in fact, the conditions of safest furnace operation demand that there shall be such an excess. This is for the following reason:

The amount of heat used in the shaft of 105 the furnace is, roughly, five or six times the amount used in the hearth. Broadly speaking, about 5,000 thermal units per pound of iron are used in the shaft and about 1,000 thermal units per pound of iron in the hearth. 110 A deficiency of a given number of thermal units would, therefore, be about five times as great, measured as a percentage, in the hearth as in the shaft. Thus, if the descending charge were short in its heat requirement by 500 thermal units to the pound of iron at the base of the shaft, this would only be a deficiency of about 10% but when the charge entered the hearth this would constitute about a 50% deficiency of the heat requirement in that region. This would be absolutely ruinous to the work of the furnace and would put it out of working commission completely. From this reasoning 115 it can be seen that it is vital that the charge shall enter the hearth without any deficiency in the heat which it should receive in the shaft and this limits radically the amount of gas which can be abstracted 120 from the base of the shaft. Generally, 125

where coke is used as the fuel in the charge, the surplus of thermal units in the shaft is considerable,—roughly speaking, from 10 per cent. up to 20 per cent., under ordinary 5 conditions. This surplus can be abstracted from the shaft without detriment to the working of the furnace. For instance, it is well known that a certain amount of water can be added to the charge without affecting 10 the work of the furnace, but if this amount be exceeded, the effect becomes highly injurious.

It will therefore be understood that in order 15 to abstract the potassium cyanid, the potassium carbonate, and the sodium compounds, and nevertheless maintain the normal operation of the furnace for its primary purpose, which is essential for commercial operations, the amount of heat abstracted 20 must be within the margin of surplus available within the shaft.

It is therefore possible to operate the furnace in either of the two ways hereinbefore described, for the recovery of the potassium 25 cyanid, potassium carbonate and sodium compounds, without upsetting the thermal equilibrium. Thus, an amount of gas within the safe margin indicated may be continuously abstracted from the bosh; or, intermittently, relatively large portions of the 30 gas may be abstracted for limited periods, the periods of withdrawal being separated by suitable time intervals, so that the drain upon the furnace shall not exceed the margin 35 of safety. Any greater abstraction than this by either method would result in upsetting the thermal equilibrium of the furnace and would cause the conditions in the hearth to pass from completely reducing to partly 40 oxidizing, owing to the presence of a considerable quantity of highly oxidizing iron oxid, which passes into the slag when the conditions in the hearth are not sufficiently reducing. This would not only upset the 45 work of the furnace and spoil the iron produced, but would probably materially reduce the amount of cyanid produced, since the oxidizing action of the slag in such case would tend to destroy it.

50 We may say further, that we regard the intermittent withdrawal of the gases for the recovery of the alkali compounds as presenting particular advantages, even in those instances where it would be feasible to withdraw 55 the gases continuously. For instance, the removal of the gases continuously involves the removal of a correspondingly small percentage of gases, per unit of time; so that there is a tendency to clog up the 60 small aperture or apertures through which the gases are withdrawn, and, at the same time, the relatively slight draft on the zone of concentration of the alkali compounds, tends to limit the withdrawal of the compounds 65 to a more or less local region in the

vicinity of the aperture or apertures. On the other hand, the intermittent operation, by permitting the accumulation of the alkali compounds up to a certain point of saturation, enables the operator to remove a 70 larger proportion of the gas, with a high percentage of the alkali compounds, during a relatively short interval, and the attendant high velocity of the withdrawn gases not only tends to prevent clogging of the apertures through which they pass, but also insures a deeper draft on the zone of concentration of the alkali compounds; so that, by the intermittent process, practised at such 75 intervals as will not disturb the thermal 80 conditions of the blast furnace, a high recovery of the alkali compounds is assured, even though the analysis of the furnace charge is relatively low in alkali.

What we claim is:

1. The method of operating iron blast furnaces, which consists in carrying on the blast furnace process to produce iron and slag as usual, and to produce by a heated air blast supplied under pressure an atmosphere of reducing gas in contact with the ignited fuel, withdrawing from the furnace such portions of the reducing gases as are not necessary for maintaining the required reducing conditions in the stack, and abstracting from said withdrawn gases the compounds of the alkali metals contained therein.

2. The method of operating iron blast furnaces, which consists in carrying on the blast furnace process to produce iron and slag as usual, and to produce by a heated air blast supplied under pressure an atmosphere of reducing gas in contact with the ignited fuel, withdrawing from the furnace such portions of the reducing gases as are not necessary for maintaining the required reducing conditions in the stack, and abstracting from said withdrawn gases the compounds of the alkali metals contained therein, the withdrawal of the reducing gases being effected at a point in their upward travel below that at which the said compounds would be precipitated or disassociated by the colder materials in the furnace.

3. The method of operating iron blast furnaces, which consists in carrying on the blast furnace process to produce iron and slag as usual, and to produce by a heated air blast supplied under pressure an atmosphere of reducing gas in contact with the ignited fuel, withdrawing from the furnace such portions of the reducing gases as are not necessary for maintaining the required reducing conditions in the stack, and abstracting from said withdrawn gases the compounds of the alkali metals contained therein, the withdrawal of the reducing gases taking place periodically so as to per-

mit the building up or accumulating of said compounds therein in the periods of time between withdrawals.

4. The method of operating iron blast furnaces, which consists in carrying on the blast furnace process to produce iron and slag as usual, and to produce by a heated air blast, supplied under pressure, an atmosphere of reducing gas in contact with the ignited fuel, regulating the operation so as to maintain slag of a light color, withdrawing from the furnace such portions of the reducing gases as are not necessary for maintaining the required reducing conditions in the stack, and abstracting from said withdrawn gases the compounds of the alkali metals contained therein.

5. The method of operating iron blast furnaces, which consists in carrying on the blast furnace process to produce iron and slag as usual, and to produce by a heated air blast, supplied under pressure, an atmosphere of reducing gas in contact with the ignited fuel, withdrawing from the furnace a portion of the reducing gases containing alkali carbonate at a rate which will not destroy the thermal equilibrium of the furnace, and abstracting from said withdrawn gases the alkali carbonate contained therein.

6. The method of operating iron blast furnaces, which consists in carrying on the blast furnace process to produce iron and slag as usual, and to produce by a heated air blast, supplied under pressure, an atmosphere of reducing gas in contact with the ignited fuel, withdrawing from the furnace

a portion of reducing gases containing a sodium compound at a rate which will not destroy the thermal equilibrium of the furnace, and abstracting from said withdrawn gases the sodium compound contained therein.

7. The method of operating iron blast furnaces, which consists in carrying on the blast furnace process to produce iron and slag as usual and to produce by a heated air blast supplied under pressure an atmosphere of reducing gas in contact with the ignited fuel, permitting the building up or accumulation of alkali compounds within said gases, and periodically withdrawing the major part of the alkali compounds thus accumulated together with such limited amount of reducing gases as will not destroy the thermal equilibrium of the furnace, and abstracting the alkali compounds from the withdrawn gases.

In testimony whereof I, HARRY B. WEAVER, affix my signature on this sixth day of August, 1918.

HARRY B. WEAVER.

Witnesses:

E. C. KOONS,  
A. E. BROWN.

In testimony whereof I, JAMES GAYLEY, affix my signature on this second day of August, 1918.

JAMES GAYLEY.

Witnesses:

WALTER S. REED,  
F. W. YOST.